

## UNITED STATES PATENT OFFICE

ADOLF KÄMPF, OF DESSAU-ZIEBIGK, GERMANY, ASSIGNOR TO I. G. FARBENINDUSTRIE AKTIENGESELLSCHAFT, OF FRANKFORT-ON-THE-MAIN, GERMANY, A CORPORATION OF GERMANY

## PRECIPITATING BATH FOR MAKING THREADS OR THE LIKE FROM VISCOSE

No Drawing. Application filed December 28, 1928, Serial No. 329,073, and in Germany January 5, 1928.

This invention relates to an improved process for making artificial threads, bands or films from viscose.

I have found that by spinning viscose, particularly unmatured viscose in a spinning bath which is substantially saturated with an organic substance of high molecular weight, particularly one having tanning properties, there are obtained threads or the like which are of high strength and extensibility, exceeding in these respects threads made when the spinning bath contains only a small proportion of such organic substance. The result is not a mere proportional effect, but is specific to the labile condition produced by the state of saturation. This is evidenced by the fact that the said state of saturation may be due to the amount of the organic substance present per se in the bath, or to the amount of the organic substance in addition to the inorganic electrolytes (acid and salts) present, in which case the percentage of the organic substance in the bath is considerably less, since the saturation state is affected by the electrolytes.

Thus it happens that with a higher concentration of acid and a smaller addition of added substance, better effects are produced on the formation of the thread than is the case with a lower acid concentration and higher addition.

The following comparison will illustrate this:—

A spinning bath which contains 15 per cent. of sulphuric acid, 17 per cent. of sodium sulfate, and such a proportion of an added substance sufficient for yielding threads which are of high luster, suffers in its good properties more or less quickly as the acid content is moderately increased, since the threads, as the content of acid rises, are more and more penetrated with bubbles which affect the physical properties and the appearance of the thread.

If, however, the acid content of the same bath is increased to a greater extent, for example to 42 per cent. the amount of sodium sulfate and organic addition which can be taken up by the bath is much smaller and amounts for example to only a small percent-

age of the quantity of acid. In spite of this, however, it is possible in a bath of such acid content to spin quite homogeneous threads of finest titer and free from included gas, and therefore very strong and lustrous, particularly when completely non-matured viscose is used.

The effect of the added organic substance is due to the formation of an adsorbed layer of the substance on the viscose threads, which layer protects the thread more or less from the weakening effect of the electrolyte. This protective layer becomes apparent when using carbazolsulfonic acid from the strong color effect of the precipitating bath on the fiber. Owing to their high tensile strength, the threads made by aid of baths according to this invention are remarkably suitable for being dyed black and for weaving silk.

The following examples illustrate the invention, the parts being by weight:—

*Example 1.*—Unmatured viscose of 5 per cent. strength and of a temperature of 9° C. is squirted into a spinning bath having a temperature of 13° C. and containing 37.5 per cent. of the artificial tanning agent being the condensation product of naphthalene sulfonic acid with formaldehyde. The individual titer is 1.4 denier, the length of immersion 70 centimeters, and the length of the path in air is 110 centimeters; the total acidity of the bath is 12 per cent calculated as sulfuric acid. The artificial silk threads produced, which are finished by the usual treatment, have a tensile strength of about 2.5 grams per denier with an extensibility of about 7 per cent.

*Example 2.*—Artificial silk is produced under the conditions described in Example 1, but by means of a precipitating bath which contains 66 parts of water 25 parts of sodium carbazolesulfonate and 9 parts of sulfuric acid. In this spinning bath threads are obtained having a tensile strength of 2.65 grams per denier and an extensibility of about 10 per cent. The threads are dyed a pronounced violet-brown.

*Example 3.*—Viscose of no degree of maturity is squirted through nozzles of 0.1 millimeter internal diameter into a bath which

contains 35 per cent. sulfuric acid and 5 per cent. of sodium carbazolesulfonate. The temperature of the bath is 13° C., the length of immersion 20 centimeters, and the rate of spinning 25 meters per minute; the wound spools are treated in a topping bath with sulfuric acid of 14.5 per cent. strength at a temperature of 6° C.

Example 4.—The same effect is produced by a bath containing 42 per cent. of sulfuric acid and 4 per cent. of sodium carbazolesulfonate. The temperature is 9° C. and the other conditions are those stated in Example 1.

Example 5.—A spinning bath is used which contains 42 per cent. of sulfuric acid and 2½ per cent. of the product of reaction of formaldehyde on naphthalene-sulfonic acid; the temperature is 6° C., the length of immersion 20 centimeters, the strength of the topping bath 14.5 per cent. of sulfuric acid, and the temperature of the topping bath 5° C.

The spinning baths specified in the preceding examples may contain an addition of 2 per cent. of sodium sulfate, and with or without this addition and also without the use of the topping bath, give good results. In all the examples the temperature of the viscose is 9° C. In each case strong and lustrous threads having good textile qualities are obtained. In using the precipitating baths according to this invention, particularly low temperatures, especially under 15° C. and also below 0° C., are of specially favorable effect.

The spinning baths according to the invention differ from those hitherto known also in the fact that by use of the additions an acid content exceeding 25 per cent. calculated as sulfuric acid may be used.

My invention is not limited to the foregoing examples or to the specific details given therein. Various modifications and changes in details and the use of equivalents of the compounds of high molecular weight enumerated in the foregoing examples are considered to be within the spirit of the invention and the scope of the following claims.

Having thus described the nature of the said invention and the best means I know of carrying the same into practical effect, I claim:

1. A process of spinning threads, bands, films and the like from viscose, particularly unmatured viscose, which comprises the step of squirting the viscose into a spinning bath containing, in a state of substantial saturation, an organic compound of high molecular weight soluble in the usual acid precipitating baths and being a tanning agent of the group consisting of carbazole sulfonic acid and formaldehyde naphthalene sulfonic acid condensation products.
65. 2. A process of producing threads, bands,

films, from viscose, particularly unmatured viscose, which comprises the step of squirting the viscose into a coagulating bath containing, in a state of substantial saturation, sodium carbazolesulfonate.

3. A process of producing threads, bands, films from viscose, particularly unmatured viscose, which comprises the step of squirting the viscose into a coagulating bath containing acid not less than 25 per cent, calculated as sulfonic acid, and, in a state of substantial saturation, an organic compound of high molecular weight soluble in the usual acid precipitating baths, of the group consisting of carbazole sulfonic acid and formaldehyde naphthalene sulfonic acid condensation products.

4. A process of producing threads, bands, films from viscose, particularly unmatured viscose, which comprises the step of squirting the viscose into a coagulating bath containing acid not less than 25 per cent, calculated as sulfonic acid, and, in a state of substantial saturation, sodium carbazolesulfonate.

5. A process of producing threads, bands, films from viscose, particularly unmatured viscose, which comprises the step of squirting the viscose into a coagulating bath containing not less than 25 per cent. of sulfuric acid and, in a state of substantial saturation, an organic compound of high molecular weight soluble in the usual acid precipitating baths, of the group consisting of carbazole sulfonic acid and formaldehyde naphthalene sulfonic acid condensation products.

6. A process of producing threads, bands, films from viscose, particularly unmatured viscose, which comprises the step of squirting the viscose into a coagulating bath containing not less than 25 per cent. of sulfuric acid and, in a state of substantial saturation, sodium carbazolesulfonate.

In testimony whereof, I affix my signature.

DR. ADOLF KÄMPF.

110

115

120

125

130

70

75

80

85

90

95

100

105

110